

C. H. F. BAGLEY.

**PROCESS FOR MAKING BASIC STEEL IN OPEN HEARTH STEEL FURNACES.**

APPLICATION FILED SEPT. 19, 1918.

1,328,803.

Patented Jan. 27, 1920.



*Inventor:*

Charles Henry Frost Bagley  
By Attorney

Fraser, Durk & Heyers

# UNITED STATES PATENT OFFICE.

CHARLES HENRY FROST BAGLEY, OF STOCKTON-UPON-TEES, ENGLAND.

PROCESS FOR MAKING BASIC STEEL IN OPEN-HEARTH STEEL-FURNACES.

1,328,803.

Specification of Letters Patent. Patented Jan. 27, 1920.

Application filed September 19, 1918. Serial No. 254,750.

To all whom it may concern:

Be it known that I, CHARLES HENRY FROST BAGLEY, of Cleveland House, Hartburn, Stockton-on-Tees, in the county of Durham, England, metallurgical engineer, have invented certain new and useful Improvements in Processes for Making Basic Steel in Open-Hearth Steel-Furnaces, of which the following is a specification.

10 This invention relates to the manufacture of basic steel in fixed open-hearth furnaces. The slag which is formed on the top of the mass of molten metal is removed from time to time by means of a blast or blasts of fluid, 15 preferably heated air or superheated steam. After such removal, further additions of lime or oxids are made.

According to this invention, the difficulties experienced, in removing the slag from a fixed furnace are entirely overcome, and where dry steam or other hot blast is employed, no serious chilling effect of the blast is incurred as regards the slag, metal and brickwork. By removing the slag in accordance with the invention, the weight of metal charged into the furnace may be increased and a greater quantity of steel produced at each heat, thereby enlarging the capacity and increasing the output of the furnace. 30 After the slag is removed by the blast, the process proceeds with greater rapidity, as there is not only a less quantity of slag to be heated to the final temperature of the steel, but also a less thickness of slag, which is a 35 poor conductor of heat, separating the flame from the metal.

The steel melting process is temporarily interrupted while the slag is being removed; but when, after the removal of the slag, 40 small fresh quantities of lime or oxids are added, they act upon the metal with greater rapidity and vigor than would otherwise be the case; so that the process as a whole is considerably expedited.

45 Moreover, a single steam or air-compressing plant is sufficient for, and may be common to, an indefinite number of furnaces, and the expense thereof, will be proportionately distributed.

50 The accompanying drawing illustrates, by way of example, an arrangement of apparatus for practising the invention, the view being a vertical cross section through the open-hearth furnace taken in the plane 55 of one of the blast twyters and slag outlets.

Referring to the drawing, *a* is the open-

hearth furnace, *b* represents molten metal and *c* the layer of slag thereon, *d* represents one of a series of twyters disposed at suitable intervals along the length of the furnace *a* at one side thereof, and supplied from an air blast trunk *e* connected to a blowing engine or the like. The twyters are made of any suitable refractory material or may be of water cooled construction, as will be well understood without further illustration, and are arranged to discharge at about the level of the slag.

At suitable intervals along the length of the other side of the furnace, slag outlets or notches *f* of usual type, are provided at positions such that when the blast is turned on to the twyters the slag is blown across the furnace and flows out through the outlets or doorways *f*.

Instead of using an air blast as illustrated, a blast of steam may be used for the purpose, suitable nozzles and steam pipes being employed instead of the air twyters and air trunk.

It will also be understood that simple perforations may be provided at a suitable angle in the brickwork, to form the blast nozzles or outlets.

Generally it is understood that I do not confine myself to the particular means described for carrying out the invention but may vary the same in detail, within the spirit of the invention.

What I claim as my invention and desire to secure by Letters Patent is:—

1. An improved process of manufacturing basic steel in fixed open hearth furnaces characterized in that the surface of metal is maintained somewhat below the lower edge of the slag holes, the slag is removed from time to time through a plurality of slag holes by means of a series of blasts of fluid acting only on a relatively small area of the surface of the metal and issuing from a plurality of twyters inclined at a suitable angle to the horizontal, and clear from close contact with the molten metal, after which further additions of lime and oxids are made which then act with great vigor and rapidity on the remaining impurities in the metal.

2. An improved process of manufacturing basic steel in fixed open hearth furnaces characterized in that the surface of metal is maintained somewhat below the lower edge of the slag holes, the slag is removed from

time to time through a plurality of slag holes by means of a series of blasts of heated fluid acting only on a relatively small area of the surface of the metal and issuing from a plurality of twyers inclined at a suitable angle to the horizontal, and clear from close contact with the molten metal, after which further additions of lime and oxids are made which then act with great vigor and rapidity on the remaining impurities in the metal.

3. An improved process of manufacturing basic steel in fixed open hearth furnaces characterized in that the surface of metal is maintained somewhat below the lower edge

of the slag holes, the slag is removed from time to time through a plurality of slag holes by means of a series of blasts of dry steam acting only on a relatively small area of the surface of the metal and issuing from a plurality of twyers inclined at a suitable angle to the horizontal, and clear from close contact with the molten metal, after which further additions of lime and oxids are made which then act with great vigor and rapidity on the remaining impurities in the metal.

In testimony whereof I have signed my name to this specification.

CHARLES HENRY FROST BAGLEY.